

## UNITED STATES PATENT OFFICE

2,098,942

PROTECTION OF MATERIALS SUBJECT TO  
PARASITIC ATTACK

Merlin Martin Brubaker, Lindemere, Del., assignor to E. I. du Pont de Nemours &amp; Company, Wilmington, Del., a corporation of Delaware

No Drawing. Application June 17, 1936, Serial No. 85,822. In Germany June 18, 1935

7 Claims. (Cl. 167—22)

This invention relates to parasiticidal compositions and more particularly to compositions containing a parasiticide and, as a fixative therefor, a basic polymeric amino-nitrogen-containing substance substantially insoluble in water and in 5 per cent aqueous ammonia, soluble in 2 per cent aqueous acetic acid and capable of being converted to a coherent film. This invention further relates to compositions of matter comprising a base material susceptible to parasitic attack having a parasiticide affixed thereto by means of an amino-nitrogen-containing polymer of the aforesaid characteristics. The invention relates further to the process of affixing and applying the parasiticide to the base material from a liquid menstruum containing said parasiticide and having dissolved therein a salt of the amino-nitrogen-containing polymer, said salt being convertible to a water insoluble substance. The invention relates more particularly to parasiticidal compositions of the aforesaid type wherein the fixative is deacetylated chitin, to the process of applying them to the base material and to the products so obtained. Whereas the art of fixing a parasiticide to a base material susceptible to parasitic attack by means of an adhesive is old and in common use, the utility of parasiticidal adhesives heretofore known has been limited by their solubility or dispersibility in water, laundering solutions, and dry-cleaning solvents and hence their utter lack of permanency toward severe rainfall, washing or dry-cleaning.

This invention has as an object the fixing or sticking of parasiticides such as stomach poisons, fungicides, bactericides, vermicides, repellents, and the like to living plant surfaces such as foliage and fruit with such a high degree of permanency as to resist for an appreciable length of time the removal of the parasiticide by heavy rainfall. A further object is the fixing of moth-proofing agents and like parasiticides to fabrics, particularly woolens, felt, fur, and like textile materials which are subject to attack by predatory insects, with such permanency that the insecticidal agents will not be removed by ordinary laundering with warm soap solutions and/or dry-cleaning with the usual dry-cleaning solvents. A still further object is to fix fungi-

cides, mildew inhibitors, mold preventatives, bactericides, and like parasiticides to fabrics, particularly cotton awnings, tents, shower bath curtains, sails, ropes, and the like materials which are ordinarily exposed to water, rain, dampness, etc., with such a high degree of resistance to such severe conditions that they retain their parasiticidal properties for long periods, when exposed to the weather, etc. Other objects will appear hereinafter.

These objects are accomplished by the following invention wherein to an object subject to parasiticidal attack, i. e. attack by fungi, insects, moths, mildew, etc., there is applied a dispersion of a parasiticide, i. e. a fungicide, insecticide, mothicide or mildew preventive, in a solution, preferably aqueous, of a salt of a polymeric amino-nitrogen containing body substantially insoluble in water and in 5% aqueous ammonia but soluble in at least the stoichiometrical amount of 2% aqueous acetic acid and capable of forming a coherent film therefrom. Deacetylated chitin is the preferred amino-nitrogen containing polymer. Others which fall under the above classification and which may be used satisfactorily are the polymeric amino alcohol methacrylates, e. g., diethylaminoethyl methacrylate polymer, the protein-amine-aldehyde condensation products, e. g., piperidylmethylein and the aminoalkyl celluloses, e. g., dimethylaminoethyl cellulose.

The unique feature of the invention, as practiced along the general lines just given, is the great resistance of the dried dispersion toward removal by attrition or handling or by rainfall, laundering or dry-cleaning as the case may be. Thus the base material susceptible to parasitic attack is rendered immune to the depredations of parasites for an indefinite period of time.

In the more detailed practice of the invention, a parasiticide (preferably a water-insoluble solid or liquid) is dispersed in an aqueous solution of a salt (preferably with a volatile acid such as acetic or formic) of a polymeric amino-nitrogen containing body which possesses the properties described hereinbefore. In some cases the proportion of polymeric amino body may be as low as 0.01 per cent with the parasiticide at a concentration of 2 per cent. These proportions may,

of course be widely varied, the ratio of polymeric amino compound to parasiticide determining the degree of permanence. Also the proportions of sticking agent necessary to attain a desired degree of permanence are different for different amino-nitrogen containing polymers and for different parasiticides. It is desirable in some cases that the parasiticide adhere not too firmly to the base as for example in the sticking of insecticides to fruits. For example, thiadiphenylamine containing about 0.5 per cent of dimethylaminomethylzein formate and made up into an approximately 2 per cent spray suspension adheres to fruit to about the correct degree. In other cases, e. g., with mothproofing agents, a higher degree of permanence is desirable. For example, a 0.5 per cent emulsion of n-dodecyl thiocyanate containing about 8 per cent of deacetylated chitin acetate based on the weight of n-dodecyl thiocyanate, when applied to woolens causes the n-dodecyl thiocyanate to be affixed thereto with the necessarily higher degree of permanency required for mothproofing.

Since the amine polymer salt is in itself a good dispersing agent for the parasiticide, additional wetting or dispersing agents while they may be added to the mixture if desired, are not essential. Whether present or not the results are satisfactory.

After the parasiticidal composition is applied to the base material, as by dipping, soaking, brushing, spraying, etc., the treated base should be thoroughly dried, either by simple exposure to the air or by forced means. Fabrics, for example, should preferably be given a heat treatment as by a calender, mangle, or pressing iron.

Any water-insoluble parasiticidal substance, either liquid or solid, that can be dispersed in an aqueous medium can be used in this invention.

For example, barium fluosilicate, "Lorol" thiocyanate, dodecyl thiocyanate, lead arsenate, thiadiphenylamine, salicylanilide, carbon bisulfide, and kerosene have been used successfully. However, the fixing agents are very definitely limited to salts, with acids, of basic amino-nitrogen containing polymeric substances which are substantially insoluble in water and 5 per cent aqueous ammonia, soluble in 2 per cent aqueous acetic acid, and capable of being converted into a coherent film. Thus the acetate of dimethylamine-phenol-formaldehyde resin, the formate of dimethylaminomethylzein, the acetate of piperidylmethylzein and, in particular, the salts of deacetylated chitin with volatile acids, e. g., acetic, have been used with a high degree of success.

The invention is not limited to the use of aqueous dispersions of parasiticides in aqueous solutions of salts of the amino-nitrogen containing polymers. In a few cases solutions of the amine polymer salts in organic solvents have been useful for fixing mothicides to fabrics. Thus, trichloroethylene solutions of the stearates of beta-dimethylaminoethyl methacrylate polymer and of methylamine-phenol-formaldehyde resin have fixed "Lorol" thiocyanate to cloth with a considerable degree of permanence. "Lorol" is a commercial product consisting of the midfraction of the long chain alcohols produced by carboxyl hydrogenation of coconut oil and consists principally of n-dodecanol.

The unique fixative properties of the salts of the hereinbefore defined polymeric amino-nitrogen containing substances are attributable to the

fact that they are strongly adsorbed on the surface of the particles of the suspended or dispersed parasiticide. As the dispersion of parasiticide dries after application to the base material, the individual particles of the parasiticidal material become coated with a continuous film or membrane of the amino-nitrogen containing polymer which either spontaneously or by heat treatment becomes insolubilized and prevents the removal of the enclosed particle by redispersion or solution. At the same time, the particle is cemented to the base material by means of that portion of the enveloping membrane which is in contact with the base material. That such an enveloping film, skin, or membrane does exist was demonstrated by an experiment involving the microscopic examination of a dried dispersion containing 0.5 per cent n-dodecyl thiocyanate and 0.04 per cent deacetylated chitin acetate. Under the microscope at a magnification of 1000 the oil droplets were easily observed. Then a drop of dodecyl thiocyanate was placed on the dried emulsion and a cover glass pressed down upon it. If the oil droplets were enveloped by a skin or membrane which has a refractive index different from the oil, the individual droplets should be observed unchanged while if no such completely enclosed film existed, they should instantly coalesce with the larger body of oil and disappear from view. However, they remained unchanged and intact demonstrating the existence of the protective film although during the course of adjustments for taking photomicrographs, two droplets were seen to disappear in a burst as if the membrane had ruptured and allowed the droplet to coalesce.

Having thus outlined the objects and principles of the invention the following exemplifications thereof are furnished for purposes of illustration and not in limitation.

*Example 1.—"Lorol" thiocyanate mothproofing emulsion*

To a solution of 1 part of deacetylated chitin in 100 parts of 2 per cent aqueous acetic acid was added 10 parts of "Lorol" thiocyanate containing 0.5 per cent of "du Pont oil red", a hydrocarbon-soluble dye having solubilities similar to those of "Lorol" thiocyanate. This mixture was emulsified in a colloid mill and diluted to 1000 parts with distilled water. White woolen flannel was impregnated with the emulsion at 80° C. for two minutes, squeezed dry, dried at room temperature, and heated at 110° C. for 1½ hours in an oven. The sample of cloth was colored a rose-red. Portions of this sample were washed and dry-cleaned several times and compared with a sample of the same cloth impregnated with a 1 per cent acetone solution of the dyed "Lorol" thiocyanate that contained no fixing agent. For each washing test the flannel was agitated and squeezed for 4 minutes in 0.3 per cent soap solution at 45° C., then washed three times in distilled water at 45° C. For each dry-cleaning, the flannel was agitated for 2 minutes at room temperature in trichloroethylene having in it 0.25 per cent of a potassium oleate soap containing 10 per cent free oleic acid, after which it was wrung out and rinsed in benzene for 1 minute. The depth of color indicated qualitatively whether the mothproofing agent was being removed by the treatments. From the results shown in Table I,

the permanence of the mothproofing composition is apparent.

not especially resistant to the dry-cleaning tests as determined qualitatively by color fading.

Table I

| Nature of treatment | Fixative | Color before treatment | Color after treatment; number of cleansing treatments |                   |                        |                    | 5  |
|---------------------|----------|------------------------|-------------------------------------------------------|-------------------|------------------------|--------------------|----|
|                     |          |                        | 1                                                     | 2                 | 3                      | 6                  |    |
| Washed.....         | Present  | Rose red               | Very slightly lighter.                                | .....             | Slightly lighter.      | No further change. | 10 |
| Dry cleaned.....    | Present  | Rose red               | No change.                                            | .....             | Very slightly lighter. | Slightly lighter.  | 10 |
| Washed.....         | Absent   | Rose red               | Very pale pink.                                       | Almost colorless. | .....                  | .....              | 15 |
| Dry cleaned.....    | Absent   | Rose red               | Colorless.                                            | .....             | .....                  | .....              | 15 |

20 *Example II.—Dodecyl thiocyanate mothproofing emulsion*

To a solution of 0.4 part deacetylated chitin, 1 part soluble aluminum acetate, 1 part acetic acid, and 0.03 part diethylcyclohexylamine 25 "Lorol" sulfate in 150 parts of water was added 5 parts dodecyl thiocyanate. This mixture was emulsified in a colloid mill and diluted with distilled water to 1000 parts. The remarkable avidity of woolen fibers for the suspended particles in 30 this emulsion was demonstrated by the following experiment:

In 50 parts of distilled water maintained at

20 *Example IV. — Thiodiphenylamine insecticidal composition*

Insecticidal sprays containing as fixatives the salts of three different amino-nitrogen containing polymers having the aforementioned properties were made up and sprayed onto glass plates, 25 dried, and subjected to 1/2 inch of artificial rainfall delivered from a spray gun in 1.4 minutes. The conditions of this test are much more severe than those which obtain under natural conditions. The results are shown in Table II along with the control and comparison with lead 30 arsenate, a naturally well-sticking insecticide.

Table II

| Insecticide        | Fixative                          | Spray composition         |                        | Deposit | Percent loss |
|--------------------|-----------------------------------|---------------------------|------------------------|---------|--------------|
|                    |                                   | Insecticide concentration | Fixative concentration |         |              |
| Thiodiphenylamine. | None                              | Percent                   |                        | Mg      |              |
| Do.....            | Deacetylated chitin acetate.      | 2                         | 0.012                  | 9.4     | 86           |
| Do.....            | Piperidylmethylzein acetate.      | 2                         | 0.01                   | 7.5     | 56           |
| Do.....            | Dimethylamino-methylzein formate. | 2                         | 0.01                   | 8.8     | 66           |
| Lead arsenate..... | None.....                         | 1                         |                        | 8.8     | 62           |
|                    |                                   |                           |                        | 5.7     | 70           |

50 80° C. there was stirred a 4.6 parts sample of woolen flannel. The above emulsion was then added slowly, with stirring, a distinct turbidity being imparted to the water. After 4 minutes of stirring the turbidity failed to clear up. A total of 8.0 parts of emulsion was added and taken up by the cloth, this representing 0.04 part of the dodecyl thiocyanate or 0.87 per cent of the weight of the cloth. This experiment indicated 55 that woolen cloth will retain at least 0.87 per cent of its weight of dodecyl thiocyanate-deacetylated chitin particles after continued washing with water.

60 *Example III.—The stearates of methylamine-phenol-formaldehyde resin and beta-diethylaminoethyl methacrylate as mothicide fixatives*

Solutions in trichloroethylene were made up 70 containing 0.2 per cent of the above stearates and 0.5 per cent of "Lorol" thiocyanate containing dye as in Example I. Woolen flannel impregnated in these solutions at about 40° C. for 1 minute, wrung out, and dried at 60-65° C. were found 75 to be fairly resistant to the washing tests but

It will be noted that all three of the amino polymer fixatives caused from two to three times as much thiodiphenylamine to be retained as was the case when no fixative was employed. It will further be noted that the deacetylated chitin is 55 definitely superior in fixative action to the two amino proteins.

60 *Example V.—Fixative for barium fluosilicate*

An aqueous dispersion containing 5 per cent barium fluosilicate and 0.5 per cent deacetylated chitin acetate was brushed on black paper and dried. The deposit was very resistant to rubbing off even when moistened, in contrast to the ease with which the barium fluosilicate was brushed off when the amine polymer salt was omitted from the formulation.

65 *Example VI.—Fixing insecticides to leaves*

An aqueous dispersion containing 0.33 per cent deacetylated chitin acetate, 0.16 per cent thiodiphenylamine, 0.16 per cent talc, and 0.007 per cent sodium dodecylsulfate was brushed on some green leaves and dried. The deposit was resistant to rubbing off after moistening.

*Example VII.—Fixing of insecticides to apples*

Several apples and apple peelings were coated with an aqueous dispersion containing 2 per cent lead arsenate and 0.1 per cent of deacetylated chitin acetate and dried thoroughly in sunlight. The deposit could be removed under running tap water only by rigorous rubbing. However, a pre-treatment with 0.5 per cent hydrochloric acid loosened the deposit so that it could easily be removed. An apple coated with a dispersion of lead arsenate alone was easily washed clean with tap water.

*Example VIII.—Mildew-proofing compositions*

A mildew-proofing dispersion was prepared containing 23.1 per cent salicylanilide, 28.9 per cent of 3.5 per cent deacetylated chitin acetate solution, and 48.0 per cent water. Samples of awning canvas were impregnated at 77-82° C. in an aqueous bath containing 10.4 lbs. of the above dispersion in 100 gals. The treated samples were then exposed to the weather for 60 days in the fall and early winter, and tested for mildew resistance by inoculation with various types of spores and storing for about two months in a warm, moist atmosphere. They were completely resistant to mildew growth both before and after weathering. Samples of the fabric treated with the same mildew inhibitor without the deacetylated chitin were resistant before weathering but not resistant to mold growth afterwards. An untreated control grew a heavy deposit of mildew both before and after weathering.

In the process of the present invention, amino-nitrogen containing substances insoluble in water and 5% aqueous ammonia but soluble in the stoichiometrical amount or more of at least 2% aqueous acetic acid and capable of forming a coherent film therefrom may be used. These may be dissolved in aqueous solutions of various acids. The use of volatile organic acids, for example, acetic and formic acids is preferred because of the greater ease of drying. In the process of drying, the salt of the fixative apparently decomposes, liberating the acid and being converted to the free amine which is water insoluble and thus causes the parasiticide, insecticide, fungicide, etc. to adhere firmly to the base. For application in water solution the salt should of course in general be water soluble. The solubility of a large number of salts of deacetylated chitin is disclosed in Rigby U. S. Patent 2,040,879. For application from organic solvents the salt used should be soluble therein as in Example III. Acids which may be employed include the following: formic, acetic, propionic, stearic, oleic, lauric, linoleic, acrylic, methacrylic, acetoacetic, adipic, maleic, malonic, acetylenedicarboxylic, lactic, glycolic, tartaric, phenylacetic, chloroacetic, mandelic, glutamic, benzoic, toluic, pyroric, 3-nitrophthalic, crotonic, benzenesulfonic, toluenesulfonic, naphthalenesulfonic, hydrochloric, hydrobromic, sulfuric, anthranilic, dichloroacetic, sebacic, citric, malic, and methylsulfuric acids. Aqueous acid solutions of most of the above may readily be prepared.

The invention has been illustrated largely in terms of deacetylated chitin. This material, which is the preferred fixing agent of the present invention, may be made as disclosed in Rigby, U. S. Patent 2,040,879. In addition there may be employed acid-soluble amino proteins which are reaction products of proteins with carbonyl compounds, such as lower aliphatic aldehydes and

ketones, and amines having less than nine carbon atoms in which the amino-nitrogen is joined to the aliphatic carbon, for example, those disclosed in Meigs copending application, Serial No. 59,643, filed January 17, 1936.

There may also be employed in this invention amino-celluloses soluble in dilute aqueous acetic acid containing an amino-nitrogen removed from the cellulose nucleus by a chain of atoms comprising at least one carbon atom, for example, those described in Hardy copending application, Serial No. 61,842, filed January 31, 1936; cellulose amines which are soluble in at least the stoichiometrical amount of dilute aqueous acetic acid and containing directly attached to the cellulosic nucleus from 0.5 to 1.5 aminonitrogen per glucose unit, for example, those described in Haskins copending application Serial No. 61,806, filed January 31, 1936; reaction products of vinyl ketone polymers with ammonia or primary amines, for example, those described in Balthis copending application Serial No. 69,725, filed March 19, 1936; the products obtained by catalytically hydrogenating resins having ketone groups at superatmospheric temperature and pressure and in the presence of ammonia or primary or secondary amine, such as those described in Greenewalt copending application, Serial No. 69,723, filed March 19, 1936; polymeric amino alcohol esters of acrylic and substituted acrylic acids, for example, those described in Harmon copending application Serial No. 21,810, filed May 16, 1935; and in Graves copending application Serial No. 21,807, filed May 16, 1935.

There may also be employed in the invention the dilute acetic acid-soluble amino-nitrogen containing resins prepared by reacting a phenol containing carbon, hydrogen, and oxygen only and having at least three unsubstituted positions in the nucleus at least two of which are ortho or para to phenolic hydroxyl, particularly those phenols conforming to the type



(where  $\text{R}_1$  and  $\text{R}_2$  are hydrogen, hydroxyl, methyol, or alkyl containing less than 3 carbon atoms), with an aldehyde (particularly formaldehyde) and a non-aromatic amine containing less than 7 carbon atoms, the molecular ratio of amine to phenol being not less than 0.5:1 and not greater than 1:1, and the molecular ratio of aldehyde to amine being greater than 1:1. Certain of the resins within this class are disclosed in copending application Serial No. 85,820, filed June 17, 1936.

Other polymeric amino-nitrogen containing resins soluble in dilute acetic acid and suitable for use in this invention include the resinous products prepared by treating polyvinyl chloroacetate with secondary aliphatic amines; resins prepared by reacting aliphatic or alicyclic ketones with formaldehyde and primary or secondary aliphatic amines; resinous products resulting from the reaction between diphenyl or other diaryl guanidine, such as diphenylguanidine, formaldehyde, and primary or secondary amines; resins prepared by reacting urea and formaldehyde with lower primary or secondary aliphatic amines such as methyl, dimethyl, butyl, and diethylamines; reaction products of epichlorohydrin with ammonia or primary aliphatic amines, which reaction products have been polymerized in the presence of catalytic proportions

5

10

15

20

25

30

35

40

45

50

55

60

65

70

75

75

of stannic chloride; the reaction product of phenol-lignin with dimethylamine and formaldehyde; and the reaction products of triethanolamine with phthalic esters, singly or in combination.

- 5 Additional examples of specific polymeric amino-nitrogen containing substances which function in this invention are dimethylaminopropyl cellulose, beta-aminoethoxyethyl cellulose, beta-dibutylaminoethyl cellulose, the mixed amino propyl-amino-propoxyethyl ether of cellulose, dibutylaminopropyl cellulose, the mixed methyldimethylaminopropyl ether of cellulose, amylnomethyl cellulose, diethylamino glycol cellulose, 10 hydroxyethylamino glycol cellulose, benzylamino methyl cellulose, diethylamino methyl cellulose, 2-hydroxycyclohexylamino methyl cellulose, amylnamino cellulose, beta-dicyclohexylaminoethyl methacrylate polymer, beta-di-n-butylaminoethyl methacrylate polymer, 2-aminocyclohexyl methacrylate polymer, triethanolamine monomethacrylate polymer, 2-(diethylamino)-cyclohexyl methacrylate polymer, beta-morpholino-N-ethyl methacrylate polymer, beta-diethylaminoethyl acrylate polymer, beta-dicyclohexylaminoethyl acrylate polymer, beta-piperidylethyl acrylate polymer, the resin obtained by the hydrogenation, in the presence of ammonia, of polymerized bis (4-ketocyclohexyl) dimethylmethane, 15 the resin resulting from the hydrogenation, in the presence of ammonia, of methylenecyclohexanone polymer, the resin obtained from the hydrogenation, in the presence of ammonia, of polymerized methylvinyl ketone, the reaction product of polymeric methyl  $\alpha$ -methylvinyl ketone and aqueous ammonia, the reaction products of polymeric methyl vinyl ketone and aqueous ammonia (or cyclohexylamine, glucamine, ethanolamine, or ethylenediamine), dimethylaminomethylzein, diethylaminomethylzein, dibutylaminomethylzein, cyclohexylethylaminomethylzein, piperazylmethylzein, piperidylmethylglycinin, dimethylaminomethylgliadin, dimethylaminoethyl-casein, monoethylaminomethylzein, the reaction product of polyvinyl chloroacetate and dibutylamine, the resin obtained by reacting cyclohexanone and formaldehyde with methylamine, the products obtained by reacting acetone and para-formaldehyde with methyl or butylamine, the 20 resin obtained by reacting diphenylguanidine and formaldehyde with methylamine, and the resins obtained by reacting urea and formaldehyde with methyl-, dimethyl-, butyl-, or dibutylamine.
- Any dispersable liquid or solid parasiticide compatible with the salts of the amino polymer may be used in this invention, among them barium fluosilicate, lead arsenate, white arsenic, n-dodecyl thiocyanate, calcium arenate, flowers of sulfur, sodium fluosilicate, aluminum fluosilicate, Paris green, mineral oils, tar distillates, vegetable oils, derris powder, nicotine sulfate, carbon bisulfide, barium carbonate, copper carbonate, calcium cyanide, copper arsenite, mercuric chloride, thiadiphenylamine, mercaptobenzothiazole, strychnine, salicylanilide, and the like. Moreover, parasiticides that are soluble in water and compatible with amine salts may be used in these parasiticidal compositions such as copper chloride, phenols, sodium cyanide, lead acetate, and the like. Also solvents other than water, such as organic hydrocarbon solvents may in some cases be used to advantage as for example in mothproofing prefabricated woolen goods, furs, etc. With these parasiticidal compositions may be combined any number of parasiticides each

having a specific function as for example a stomach poison insecticide may be combined with a fungicide and/or a contact insecticide for controlling a number of different pests at once. Also like compositions may be of advantage in fixing 5 herbicides to pestiferous plants such as weeds, to effect their extermination.

The components of the compositions of this invention may be applied to the base material separately in two or more steps or operations, the 10 solution of the basic amino polymer preferably though not necessarily being applied last. Other ingredients may also be added to these compositions such as dyes, pigments, softening agents, water repellent waxes, sizing materials, wetting 15 agents, dispersing agents, etc., and the compositions may be used in connection with various textile finishing operations, plant treatments, and the like.

The compositions containing a parasiticide and 20 a fixative comprising a polymeric amino-nitrogen containing substance have been found useful for mothproofing woolen goods with a high degree of permanence, the mothproofing agent being fixed to the fibers with such firmness as to resist 25 removal by laundering and dry cleaning. The compositions are useful for fixing insecticides to plant surfaces which are susceptible to parasitic attack such as the foliage and fruit. These insecticidal compositions are resistant to removal 30 by severe rainfall. These compositions have also been found to be highly useful for fixing mildew inhibitors such as salicylanilide to cotton fabrics with such a high degree of tenacity that severe 35 weathering or washing does not destroy their fungicidal properties. The compositions are highly useful for the purpose of fixing any parasiticide to any base material such as wood, cloth, paper, fur, hair, a living plant or animal surface, and the like, which is susceptible to parasitic attack and which must withstand washing, dry-cleaning or rainfall.

Parasiticidal stickers or adhesives previously used comprising glue, gelatin, gum arabic, gum dammar, casein, albumin, dextrine, and similar 45 hydrophylic colloidal substances suffer the disadvantage of being readily redissolved or redispersed by water or soap solutions and for this reason they are completely ineffective when exposed to rainfall, dampness, or laundering. Oils, waxes, 50 and resins may be easily removed as a rule by detergents such as soap and by dry-cleaning solvents. By the use of salts of amino-nitrogen containing resins which are insoluble in water and dilute alkali but soluble in dilute acids, the 55 parasiticide is anchored to the base material by a film which when thoroughly dry becomes water-insoluble and non-dispersable by alkaline or soap solutions because of the evaporation of the volatile acid which is preferably used, such as acetic or formic acid. While in some cases the film may be redispersed by dilute acid solution, in other cases it cannot, due to further polymerization of the amine polymer under the drying conditions. Thus the adhesive substance in the parasiticidal compositions fixes the parasiticide to the base material with real permanence toward rainfall, laundering and dry-cleaning.

A further advantage is that very small proportions of the fixative are required (0.5 per cent 70 to 8 per cent of the weight of parasiticide) as against the large proportions (40 to 100 per cent of the weight of parasiticide) needed with the old type of sticker such as dextrine. Thus the efficiency of the parasiticide is not lowered.

Fluosilicates and similar fluoro anion salts of amino-nitrogen-containing polymeric bodies substantially insoluble in water and in 5% aqueous ammonia but soluble in 2% aqueous acetic acid and capable of being converted to a coherent film, as well as solutions of these salts and the use of these solutions in protecting materials from parasitic attack are disclosed and claimed in copending application Serial No. 116,435, filed December 10, 1936 by Paul L. Salzberg.

The term parasite, as used in the specification and claims, is thus used to include not only bacteria, fungi, insects and other small animal life preying on living organism but in a wider sense to include also fungi and bacteria even when no longer attacking living matter, moths, molds and other forms of harmful minute life harmful to animal or vegetable matter even when this matter is no longer living.

The term parasiticide has a similar scope and therefore includes vermicides, contact insecticides, stomach poisons, herbicides, mothcides, mildew preventives, mold preventives, bactericides, etc.

The above description and examples are intended to be illustrative only. Any modification or variation therefrom which conforms to the spirit of the invention is intended to be included within the scope of the claims.

I claim:

1. A composition of matter suitable for protecting materials against parasitic attack comprising a dispersion of a parasiticide in a solution of a salt of a polymeric amino-nitrogen containing body substantially insoluble in water and in 5% aqueous ammonia but soluble in at least the stoichiometrical amount of 2% aqueous acetic

acid and capable of forming a coherent film therefrom.

2. A composition of matter suitable for protecting materials against parasitic attack comprising a dispersion of a parasiticide in an aqueous solution of a salt of a polymeric amino-nitrogen containing body substantially insoluble in water and in 5% aqueous ammonia but soluble in at least the stoichiometrical amount of 2% aqueous acetic acid and capable of forming a coherent film 10 therefrom.

3. A composition of matter suitable for protecting materials against parasitic attack comprising a dispersion of a parasiticide in an aqueous solution of a salt of deacetylated chitin.

4. A composition of matter suitable for protecting materials against parasitic attack comprising a dispersion of a parasiticide in an aqueous solution of an acetate of deacetylated chitin.

5. A composition of matter comprising a base 20 material susceptible to parasitic attack having a parasiticide affixed thereto by means of an amino-nitrogen containing polymeric body substantially insoluble in water and in 5% aqueous ammonia, soluble in 2% aqueous acetic acid and capable of 25 being converted to a coherent film.

6. A composition of matter comprising a base material susceptible to parasitic attack having a parasiticide affixed thereto by means of deacetylated chitin.

7. A composition suitable for protecting fabrics against fungus attack comprising salicylanilide dispersed in an aqueous solution of an acetate of deacetylated chitin.

MERLIN MARTIN BRUBAKER. 35